# EUROPEAN PATENT SPECIFICATION

(11) **EP 2 304 000 B1**
(45) Date of publication and mention of the grant of the patent: **05.08.2020**
(21) Application number: 09772459.5
(22) Date of filing: 30.06.2009
(51) Int. Cl.: C10L 1/19, C10L 10/10

(54) **GASOLINE COMPOSITIONS**
BENZINZUSAMMENSETZUNGEN
COMPOSITIONS D'ESSENCE

(30) Priority: 02.07.2008 EP 08159554
(43) Date of publication of application: 06.04.2011
(73) Proprietor: Shell Internationale Research Maatschappij B.V., 2596 HR The Hague (NL)
(72) Inventor: CLARKE, Lionel, Chester Cheshire CH2 4NU (GB); FELIX-MOORE, Alison, Chester Cheshire CH2 4NU (GB); LOUIS, Jurgen Johannes Jacobus, 21107 Hamburg (DE); SMITH, Johanne, Chester Cheshire CH2 4NU (GB); LANGE, Jean-Paul, 1031 HW Amsterdam (NL)
(74) Representative: Shell Legal Services IP
(86) International application number: PCT/EP2009/058226
(87) International publication number: WO 2010/000759

(56) References cited:
- AU-A1- 2003 252 892
- US-A1- 2001 034 966
- US-B1- 6 679 302

## Description

### Field of the Invention

The present invention provides a method of controlling the vapour pressure of a gasoline.

### Background of the Invention

Ethyl valerate (also called ethyl pentanoate) is an ester commonly used in fragrance and flavouring applications.

JP57-115490-A1 (K.K. My-Skincare-Laboratories & Daikyu K.K.) discloses a kerosene deodoriser containing 1 kind or 2 or more kinds of lower fatty acid esters. Ethyl esters of valeric acid are included in the description as examples of possible lower fatty acid esters.

JP07-018269-A1 (Riken Koryo Kogyo K.K.) discloses fuel additives for suppressing the unpleasant odour characteristic of the fuel produced during incomplete combustion of said fuel. Ethyl pentanoate is disclosed as an ester useful as an odour suppressing additive, and gasoline compositions comprising 0.2 wt.% ethyl pentanoate are disclosed therein.

WO 01/36354 A1 (Ronyak) discloses compositions containing an odour-emitting hydrocarbonaceous material and an odour-suppressing amount of an aldehyde or a ketone, and a carboxylic acid ester. Ethyl valerate is disclosed as a carboxylic acid ester (Claim 18) and gasoline is disclosed as an odour-emitting hydrocarbonaceous material (Claim 9).

US 2,228,662 and US 2,334,006 (Standard Oil Company) discloses the addition of esters to motor fuels consisting essentially of branched chain paraffin hydrocarbons and having a relatively high anti-knock value to increase the anti-knock quality thereof.

The motor fuels to which the ester is added in both US 2,228,662 and US 2,334,006 is described as "consisting essentially of branched chain paraffin hydrocarbons, and more specifically describes the base fuel to which the ester is added as branched chain paraffin stocks comprising from five to twelve carbon atoms per molecule. US 2,228,662 and US 2,334,006 further describe that the base fuel of invention disclosed therein "usually is not alone a satisfactory motor fuel, for it is usually necessary that more volatile constituents, such as natural gasoline for example, be blended with it to make a finished fuel having the desired volatility or distillation curve, so that the fuel will have the desired characteristics relating to starting, acceleration, etc.", and that such blending is objectionable because the more volatile blending stocks usually have relatively low anti-knock values.

US 2,228,662 and US 2,334,006 discloses that many of the esters "aid in producing a motor fuel having the desired volatility or distillation characteristics and reduce, and in some cases even eliminate, the proportion of volatile constituents". US 2,228,662 and US 2,334,006 further discloses that esters containing four or five carbon atoms have "relatively high volatility", and that esters containing three carbon atoms may be used "where higher volatility is desired" and esters containing six to seven carbon atoms per molecule where "relatively low volatility offers no problem". However, the person skilled in the art would understand from US 2,228,662 and US 2,334,006 that the base motor fuels described therein have a volatility that is undesirably low for use as a motor fuel and that more volatile constituents need to be blended with it to make a finished fuel having suitable volatility.

Neither US 2,228,662 or US 2,334,006 quantify nor exemplify the effects on the volatility on the motor fuels disclosed therein caused by the addition of the esters disclosed therein.

The person skilled in the art would understand from the disclosures of US 2,228,662 and US 2,334,006 that esters may be used to increase the volatility of motor fuels having a volatility that is undesirably low, and that esters containing 3 carbon atoms increase the volatility of the motor fuel more than the esters containing six or seven carbon atoms.

US 2001/0034966 A1 discloses a method of reducing the vapour pressure of a C₃ to C₁₂ hydrocarbon-based motor fuel mixture containing 0.1 to 20 % by volume of ethanol for conventional spark ignition internal combustion engines, wherein, in addition to an ethanol component (b) and a C₃ to C₁₂ hydrocarbon component (a), an oxygen-containing additive (c) selected from at least one of the following types of compounds: alcohol other than ethanol, ketone, ether, ester, hydroxy ketone, ketone ester, and a heterocyclic containing oxygen, is used in the fuel mixture in an amount of at least 0.05 by volume of the total fuel.

The vapour pressure of a fuel (e.g. Air Saturated Vapour Pressure (ASVP), Dry Vapour Pressure Equivalent (DVPE) or Reid Vapor Pressure (RVP)) is a measure of the volatility of the motor fuel. Fuels having a high vapour pressure may vaporise too readily in the fuel handling system, resulting in decreased flow to the engine and possibly stoppage through vapour lock. Conversely, fuels having low vapour pressure may not vaporise readily enough, resulting in difficulty starting (especially in winter conditions), slow warm-up and poor acceleration.

Surprisingly, we have found that, contrary to the teachings of US 2,228,662 and US 2,334,006, the use of ethyl valerate in modern gasoline fuel compositions actually causes a significant decrease in the vapour pressure of the finished fuel composition.

### Summary of the Invention

The present invention further provides a method for controlling the vapour pressure of a gasoline composition consisting of admixing with a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component, wherein the gasoline base fuel consists of a mixture of hydrocarbons boiling in the range from 25 to 230°C according to EN ISO 3405,
such that the numerical value of the vapour pressure for the gasoline composition can be numerically decreased, have no numerical change, or numerically increased relative to the numerical value of the vapour pressure for the gasoline base fuel.

The present invention further provides a gasoline composition having a Dry Vapour Pressure Equivalent (DVPE) in the range of from 30 to 110 kPa, consisting of a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component, wherein the gasoline base fuel consists of a mixture of hydrocarbons boiling in the range from 25 to 230°C according to EN ISO 3405.

The present invention yet further provides a method of operating a spark-ignition internal combustion engine, which method involves introducing into a combustion chamber of the engine a gasoline composition of the present invention.

The present invention yet further provides use of ethyl valerate and a C3-4 hydrocarbon component for controlling the vapour pressure of a gasoline composition wherein the gasoline composition consists of a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component, wherein the gasoline base fuel consists of a mixture of hydrocarbons boiling in the range from 25 to 230°C according to EN ISO 3405, such that the numerical value of the vapour pressure for the gasoline composition can be numerically decreased, have no numerical change, or numerically increased relative to the numerical value of the vapour pressure for the gasoline base fuel.

### Detailed Description of the Invention

The gasoline base fuel consists of a liquid hydrocarbon fuel and would normally be suitable for use in an internal combustion engine of the spark ignition (petrol) type. Gasolines contain mixtures of hydrocarbons boiling in the range from 25 to 230 °C (EN-ISO 3405), the optimal ranges and distillation curves typically varying according to climate and season of the year.

The hydrocarbons in a gasoline fuel may conveniently be derived in known manner from straight-run gasoline, synthetically-produced aromatic hydrocarbon mixtures, thermally or catalytically cracked hydrocarbons, hydrocracked petroleum fractions, catalytically reformed hydrocarbons or mixtures of these.

The research octane number (RON) of the gasoline base fuel may suitably be from 80 to 100, preferably from 90 to 100, more preferably from 94 to 100 (EN 25164). Its motor octane number (MON) may suitably be from 80 to 100, preferably from 84 to 100 (EN 25163).

It may have an olefin content of for instance from 0 to 20 % v/v (ASTM D1319), an aromatics content of for instance from 0 to 50 % v/v (ASTM D1319) and in particular a benzene content of at most 1 % v/v.

The base fuel, and suitably also the overall fuel composition, preferably has a low or ultra low sulphur content, for instance at most 1000 ppmw (parts per million by weight), preferably no more than 500 ppmw, more preferably no more than 100, even more preferably no more than 50 and most preferably no more than even 10 ppmw. It also preferably has a low total lead content, such as at most 0.005 g/l, most preferably being lead free- having no lead compounds added thereto (i.e. unleaded).

The gasoline composition of the present invention is produced by admixing a gasoline base fuel with ethyl valerate and a C₃₋₄ hydrocarbon component.

The ethyl valerate admixed with the gasoline base fuel in the present invention is present in a concentration in the range of from 2 vol.% to 20 vol.%, based on the total volume of the gasoline composition. The ethyl valerate admixed with the gasoline base fuel in the present invention may be present in various concentration ranges having a lower limit of from 2 vol.%, and an upper limit of at most 20 vol.%, preferably 15 vol.%, based on the total volume of the gasoline composition (e.g. 2 - 20 vol.%, and 2 - 15 vol.%).

The C₃₋₄ hydrocarbon component of the gasoline compositions of the present invention comprises C₃ hydrocarbons, C₄ hydrocarbons and mixtures thereof. Preferably, the C₃₋₄ hydrocarbon component comprises propane, butane and mixtures thereof. Conveniently, butane gas may be used as the C₃₋₄ hydrocarbon component. The C₃ and C₄ hydrocarbons present in the C₃₋₄ hydrocarbon component are in addition to any C₃ and C₄ hydrocarbons that may be present in the gasoline base fuel.

The C₃₋₄ hydrocarbon component admixed with the gasoline base fuel in the present invention may be present in a concentration in the range upwardly to 5 vol.%. The C₃₋₄ hydrocarbon component is present in the gasoline composition of the present invention in a concentration range having a lower limit of from 0.5 vol.%, and an upper limit of at most 5 vol.%, based on the total volume of the gasoline composition.

Whilst the concentration of the C₃₋₄ hydrocarbon component is typically in addition to any C₃ and C₄ hydrocarbons present in the gasoline base fuel, in one embodiment of the present invention, the amount of the C₃₋₄ hydrocarbon component in the gasoline composition is the total amount of C₃ and C₄ hydrocarbons present in the overall gasoline composition. Therefore, the gasoline composition of the present invention consists of a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component. The total amount of C₃₋₄ hydrocarbon component present in the above gasoline composition (i.e. the combined total of the C₃₋₄ hydrocarbon component and any C₃ and C₄ hydrocarbons present in the base gasoline) is in a concentration range having a lower limit of from 0.5 vol.%, and an upper limit of at most 5 vol.%, based on the overall gasoline composition.

By decreasing, reducing or lowering the vapour pressure of the gasoline base fuel, it is meant that the numerical value of the vapour pressure (e.g. ASVP, DVPE or RVP) for the gasoline compositions produced by the method of the present invention is numerically decreased relative to the numerical value of the vapour pressure for the gasoline base fuel used in the preparation of the gasoline composition according to the present invention.

Therefore, disclosed herein is the use of ethyl valerate in a gasoline composition comprising a major proportion of gasoline base fuel for reducing the vapour pressure of the gasoline composition relative to the vapour pressure of the gasoline base fuel.

Since C₃ and/or C₄ hydrocarbons are highly volatile and have a tendency to increase the vapour pressure of gasoline, the addition of the C₃₋₄ hydrocarbon component advantageously allows a greater control of the vapour pressure of the gasoline composition. Therefore, when the gasoline composition of the present invention has the C₃₋₄ hydrocarbon component admixed therein, the vapour pressure of the gasoline composition of the present invention can be controlled.

By controlling the vapour pressure of the gasoline composition, it is meant that the numerical value of the vapour pressure (e.g. ASVP, DVPE or RVP) for the gasoline compositions produced by the method of the present invention can be numerically decreased, have no numerical change, or numerically increased relative to the numerical value of the vapour pressure for the gasoline base fuel used in the preparation of the gasoline composition according to the present invention.

The DVPE of the gasoline composition of the present invention is in the range of from 30.0 kPa to 110.0 kPa, preferably in the range of from 40.0 kPa to 95.0 kPa, more preferably in the range of from 45.0 to 90.0.

The optimal vapour pressure of the gasoline compositions of the present invention will vary depending upon the climate and season of the year. For example, the optimal vapour pressure for gasoline compositions for use in hot climates would be lower than the optimal vapour pressure for gasoline compositions for use in cold climates, and the optimal vapour pressure for gasoline compositions for use in summer would be lower than the optimal vapour pressure for gasoline compositions for use in winter.

For example, summer blend gasoline compositions in Europe typically have a DVPE in the range of from 45.0 to 60.0, and winter blend gasoline compositions in Europe typically have a DVPE in the range of from 60.0 to 90.0.

Usefully, ethyl valerate can be admixed with gasoline base fuels having a vapour pressure that is above optimal for the climate or season, or is too high to meet local regulatory standards, in order to decrease the vapour pressure to be optimal for the climate or season or to meet local regulatory standards. For instance, ethyl valerate may be admixed with a seasonal gasoline formulated for use in the winter to provide a seasonal gasoline composition suitable for use in the summer.

Additionally, because gasoline compositions comprising ethyl valerate have a lower vapour pressure compared to the gasoline base fuel to which ethyl valerate has been added, the use of ethyl valerate in gasoline compositions allow the inclusion of highly volatile components in gasoline base fuels that would otherwise be prevented due to the effects on the vapour pressure of the gasoline base fuel.

Also, ethyl valerate and the C₃₋₄ hydrocarbon component can be admixed with gasoline base fuels having a vapour pressure that is above or below optimal for the climate or season, or is too high or too low to meet local regulatory standards, in order to decrease or increase the vapour pressure to be optimal for the climate or season or to meet local regulatory standards. Furthermore, ethyl valerate and the optional C₃₋₄ hydrocarbon component can be admixed with a gasoline base fuel already having an optimal vapour pressure in order to blend in to the gasoline composition excess C₃₋₄ hydrocarbons that may be produced at the refinery without causing adverse effect on the vapour pressure of the gasoline composition.

The present invention further provides a method of operating a spark-ignition internal combustion engine, which method involves introducing into a combustion chamber of the engine a gasoline composition according to the present invention.

The present invention will be further understood from the following examples, which illustrate the effects of ethyl valerate on the vapour pressure of a gasoline base fuel.

### Examples

The vapour pressures of the gasoline base fuels and gasoline compositions were tested in accordance with test method IP 394, using a SETAVAP 2 instrument.

The test involves injecting the sample (which has been pre-cooled to between 0 °C and 1 °C and air-saturated) into the test chamber, which is set to 37.8 °C +/- 0.1 °C. The pressure indicator reading is recorded every 60 s +/-5 s until 3 successive readings agree to within 0.1 kPa. The average (mean) of these 3 values is recorded as the ASVP (Air Saturated Vapour Pressure). The DVPE is then calculated from the ASVP using the equation detailed in test method IP 394.

Details of the gasoline blends are given in Table 1 below.

**Table 1**

| Example | Gasoline base fuel (%vol.) | Ethyl Valerate (%vol.) |
|---|---|---|
| A* | A (100) | - |
| 1* | A (95) | 5 ^{a} |
| B* | B (100) | - |
| 2* | B (90) | 10 ^{b} |
| 3* | B (80) | 20 ^{b} |
| C* | C (100) | - |
| 4* | C (90) | 10 ^{c} |
| 5* | C (80) | 20 ^{c} |
| D* | D (100) | - |
| 6* | D (90) | 10 ^{c} |
| 7* | D (80) | 20 ^{c} |
| E* | E (100) | - |
| 8* | E (90) | 10 ^{c} |
| 9* | E (80) | 20 ^{c} |

| | | |
|---|---|---|
| * - not according to the invention a= Ethyl valerate supplied by Aldrich (99% grade) b= Ethyl valerate supplied by Aldrich (98% grade) c= Ethyl valerate supplied by Shanghai Pu Jie, China | | |

Details of the gasoline base fuels used in the examples are given below.

Gasoline base fuel A is an unleaded gasoline base fuel (ULG-95) having the following characteristics; sulphur content (ISO 20884) 28 ppmw, aromatics content of 34.6% v/v and olefins content of 18 % v/v (GC analysis; LTP/36), density at 15 °C (IP 365) 746.5 kg/m³, and distillation (IP 123): IBP 32.8 °C, 10% 51.0 °C, 50% 100.2 °C, 90% 160.4 °C and FBP 203.0 °C.

Gasoline base fuel B is an unleaded gasoline base fuel (ULG-95) having the following characteristics; sulphur content (ISO 20884) 30.7 ppmw, aromatics content of 35.02% v/v and olefins content of 14.64 % v/v (GC analysis; LTP/36), density at 15 °C (IP 365) 742.6 kg/m³, and distillation (IP 123): IBP 30.2 °C, 10% 46.1 °C, 50% 102.1 °C, 90% 159.5 °C and FBP 202.0 °C.

Gasoline base fuel C is an unleaded gasoline base fuel (92.5 RON (ASTM D2699), 83.9 MON (ASTM D2700)) having the following characteristics; density at 15 °C (ISO 3675) 0.7431 kg/l, and distillation (IP 123): IBP 36 °C, 10% 51.3 °C, 50% 80.8 °C, 90% 154.1 °C and FBP 193.1 °C.

Gasoline base fuel D is an unleaded gasoline base fuel (94.2 RON (ASTM D2699), 84.3 MON (ASTM D2700)) having the following characteristics; density at 15 °C (ISO 3675) 0.7511 kg/l, and distillation (IP 123): IBP 35.4 °C, 10% 53.0 °C, 50% 86.4 °C, 90% 157.6 °C and FBP 198.2 °C.

Gasoline base fuel E is an unleaded gasoline base fuel (93.7 RON (ASTM D2699), 85.9 MON (ASTM D2700)) having the following characteristics; density at 15 °C (ISO 3675) 0.7534 kg/l, and distillation (IP 123): IBP 37.6 °C, 10% 59.4°C, 50% 100.2°C, 90% 157.0°C and FBP 196.0 °C.

The DVPE for each of the gasoline blends detailed in Table 1 are given in Table 2 below.

**Table 2**

| Example | Ethyl valerate (vol.%) | DVPE (Kpa) (IP 394) |
|---|---|---|
| A* | 0 | 67.7 |
| 1* | 5 | 64.9/63.4 |
| B* | 0 | 81.7 |
| 2* | 10 | 76.2 |
| 3* | 20 | 70.1 |
| C* | 0 | 56.5 |
| 4* | 10 | 54.9 |
| 5* | 20 | 51.0 |
| D* | 0 | 56.7 |
| 6* | 10 | 52.7 |
| 7* | 20 | 50.4 |
| E* | 0 | 46.6 |
| 8* | 10 | 44.4 |
| 9* | 20 | 42.1 |

It can be seen from Table 2 above that the addition of EV to base gasoline causes a decrease in DVPE relative to the gasoline base fuel, with increasing concentration of EV producing a greater decrease in the DVPE.

## Claims

1. A method for controlling the vapour pressure of a gasoline composition consisting of admixing with a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component, wherein the gasoline base fuel consists of a mixture of hydrocarbons boiling in the range from 25 to 230°C according to EN ISO 3405, such that the numerical value of the vapour pressure for the gasoline composition can be numerically decreased, have no numerical change, or numerically increased relative to the numerical value of the vapour pressure for the gasoline base fuel.

2. A method according to Claim 1 wherein butane gas is used as the C₃₋₄ hydrocarbon component.

3. A gasoline composition having a Dry Vapour Pressure Equivalent (DVPE) in the range of from 30 to 110 kPa (according to IP 394), consisting of a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component, wherein the gasoline base fuel consists of a mixture of hydrocarbons boiling in the range from 25 to 230°C according to EN ISO 3405.

4. A gasoline composition according to Claim 3 wherein butane gas is used as the C₃₋₄ hydrocarbon component.

5. A method of operating a spark-ignition internal combustion engine, which method involves introducing into a combustion chamber of the engine a gasoline composition according to claim 3 or 4.

6. Use of ethyl valerate and a C3-4 hydrocarbon component for controlling the vapour pressure of a gasoline composition wherein the gasoline composition consists of a gasoline base fuel, from 2 to 20 vol.%, based on the overall gasoline composition, of ethyl valerate, and from 0.5 to 5 vol.%, based on the overall gasoline composition, of a C₃₋₄ hydrocarbon component, wherein the gasoline base fuel consists of a mixture of hydrocarbons boiling in the range from 25 to 230°C according to EN ISO 3405,
such that the numerical value of the vapour pressure for the gasoline composition can be numerically decreased, have no numerical change, or numerically increased relative to the numerical value of the vapour pressure for the gasoline base fuel.

7. Use according to Claim 6 wherein butane gas is used as the C₃₋₄ hydrocarbon component.

## Patentansprüche

1. Verfahren zur Steuerung des Dampfdrucks einer Benzinzusammensetzung, bestehend aus dem Mischen von 2 bis 20 Vol.-% Ethylvalerat, bezogen auf die gesamte Benzinzusammensetzung, und 0,5 bis 5 Vol.-%, bezogen auf die gesamte Benzinzusammensetzung, einer C₃₋₄-Kohlenwasserstoff-Komponente, wobei der Kraftstoff auf Benzinbasis aus einer Mischung von Kohlenwasserstoffen besteht, die gemäß EN ISO 3405 im Bereich von 25 bis 230 °C sieden, sodass der numerische Wert des Dampfdrucks für die Benzinzusammensetzung numerisch verringert werden kann, keine numerische Änderung aufweist oder relativ zum numerischen Wert des Dampfdrucks für den Kraftstoff auf Benzinbasis numerisch erhöht werden kann.

2. Verfahren nach Anspruch 1, wobei Butangas als C₃₋₄-Kohlenwasserstoff-Komponente verwendet wird.

3. Benzinzusammensetzung mit einem Trockendampfdruckäquivalent (DVPE) im Bereich von 30 bis 110 kPa (gemäß IP 394), bestehend aus einem Kraftstoff auf Benzinbasis, 2 bis 20 Vol.-%, bezogen auf die gesamte Benzinzusammensetzung, Ethylvalerat und 0,5 bis 5 Vol.-%, bezogen auf die gesamte Benzinzusammensetzung, einer C₃₋₄-Kohlenwasser-Stoffkomponente, wobei der Kraftstoff auf Benzinbasis aus einem Gemisch von Kohlenwasserstoffen besteht, die gemäß EN ISO 3405 im Bereich von 25 bis 230°C sieden.

4. Benzinzusammensetzung nach Anspruch 3, wobei Butangas als C₃₋₄-Kohlenwasserstoff-Komponente verwendet wird.

5. Verfahren zum Betreiben eines Verbrennungsmotors mit Fremdzündung, wobei das Verfahren das Einleiten einer Benzinzusammensetzung nach Anspruch 3 oder 4 in eine Brennkammer des Motors umfasst.

6. Verwendung von Ethylvalerat und einer C₃₋₄-Kohlenwasserstoff-Komponente zur Steuerung des Dampfdrucks einer Benzinzusammensetzung, wobei die Benzinzusammensetzung aus einem Kraftstoff auf Benzinbasis, 2 bis 20 Vol.-%, bezogen auf die gesamte Benzinzusammensetzung, Ethylvalerat und 0,5 bis 5 Vol.-%, bezogen auf die gesamte Benzinzusammensetzung, einer C₃₋₄-Kohlenwasserstoff-Komponente besteht, wobei der Kraftstoff auf Benzinbasis aus einem Gemisch von Kohlenwasserstoffen besteht, die gemäß EN ISO 3405 im Bereich von 25 bis 230°C sieden, sodass der numerische Wert des Dampfdrucks für die Benzinzusammensetzung numerisch verringert werden kann, keine numerische Änderung aufweist oder relativ zum numerischen Wert des Dampfdrucks für den Kraftstoff auf Benzinbasis numerisch erhöht werden kann.

7. Verwendung nach Anspruch 6, wobei Butangas als C₃₋₄-Kohlenwasserstoff-Komponente verwendet wird.

## Revendications

1. Procédé permettant de contrôler la pression de vapeur d'une composition d'essence consistant à mélanger avec un carburant à base d'essence, de 2 à 20 % en volume, sur la base de la composition globale d'essence, de valérate d'éthyle, et de 0,5 à 5 % en volume, sur la base de la composition globale d'essence, d'un composant hydrocarboné en C₃₋₄, le carburant à base d'essence étant constitué d'un mélange d'hydrocarbures dont le point d'ébullition est compris entre 25 et 230 °C selon la norme EN ISO 3405, de sorte que la valeur numérique de la pression de vapeur pour la composition d'essence peut être numériquement diminuée, ne pas avoir de changement numérique, ou être numériquement augmentée par rapport à la valeur numérique de la pression de vapeur pour le carburant à base d'essence.

2. Procédé selon la revendication 1, dans lequel le gaz butane est utilisé comme composant hydrocarboné en C₃₋₄.

3. Composition d'essence ayant un équivalent de pression de vapeur sèche (DVPE) dans la plage allant de 30 à 110 kPa (selon la norme IP 394), constituée d'un carburant à base d'essence, de 2 à 20 % en volume, sur la base de la composition globale d'essence, de valérate d'éthyle, et de 0,5 à 5 % en volume, sur la base de la composition globale d'essence, d'un composant hydrocarboné en C₃₋₄, le carburant à base d'essence étant constitué d'un mélange d'hydrocarbures dont le point d'ébullition est compris entre 25 et 230 °C selon la norme EN ISO 3405.

4. Composition d'essence selon la revendication 3, dans laquelle le gaz butane est utilisé comme composant hydrocarboné en C₃₋₄.

5. Procédé de fonctionnement d'un moteur à combustion interne à allumage commandé, ledit procédé consiste à introduire dans une chambre de combustion du moteur une composition d'essence selon la revendication 3 ou 4.

6. Utilisation de valérate d'éthyle et d'un composant d'hydrocarbure en C₃₋₄ pour contrôler la pression de vapeur d'une composition d'essence dans laquelle la composition d'essence consiste en un carburant à base d'essence, de 2 à 20 % en volume, sur la base de la composition globale d'essence, de valérate d'éthyle, et de 0,5 à 5 % en volume, sur la base de la composition globale d'essence, d'un composant hydrocarboné en C₃₋₄, le carburant à base d'essence étant constitué d'un mélange d'hydrocarbures dont le point d'ébullition est compris entre 25 et 230 °C selon la norme EN ISO 3405, de sorte que la valeur numérique de la pression de vapeur pour la composition d'essence peut être numériquement diminuée, ne pas avoir de changement numérique, ou être numériquement augmentée par rapport à la valeur numérique de la pression de vapeur pour le carburant à base d'essence.

7. Utilisation selon la revendication 6, dans laquelle le gaz butane est utilisé comme composant hydrocarboné en C₃₋₄.
